

# United States Patent [19]

Normandin et al.

[11] Patent Number: 4,942,117

[45] Date of Patent: Jul. 17, 1990

[54] PHOTOGRAPHIC SILVER HALIDE MATERIALS AND PROCESS COMPRISING A PYRAZOLOAZOLE COUPLER

[75] Inventors: **Sharon E. Normandin**, Macedon; **Arlyce T. Bowne**, Rochester, both of N.Y.; **Nigel E. Milner**; **David Clarke**, both of Watford, Great Britain

[73] Assignee: **Eastman Kodak Company**, Rochester, N.Y.

[21] Appl. No.: 412,722

[22] Filed: Sep. 26, 1989

## Related U.S. Application Data

[63] Continuation-in-part of Ser. No. 171, 061, Mar. 21, 1988, abandoned, which is a division of Ser. No. 23, 517, Mar. 9, 1987, abandoned.

[51] Int. Cl.<sup>5</sup> ..... G03C 7/38

[52] U.S. Cl. ..... 430/558; 430/386; 430/387; 430/476

[58] Field of Search ..... 430/558, 386, 387, 476

## References Cited

### U.S. PATENT DOCUMENTS

|           |        |                  |       |         |
|-----------|--------|------------------|-------|---------|
| 4,338,393 | 7/1982 | Bailey et al.    | ..... | 430/387 |
| 4,443,536 | 4/1984 | Lestina          | ..... | 430/552 |
| 4,540,654 | 9/1985 | Sato et al.      | ..... | 430/381 |
| 4,600,688 | 7/1986 | Kawakatsu et al. | ..... | 430/558 |
| 4,607,002 | 8/1986 | Nakayama et al.  | ..... | 430/505 |
| 4,639,415 | 1/1987 | Kaneko et al.    | ..... | 430/558 |
| 4,684,603 | 8/1987 | Nishijima et al. | ..... | 430/558 |

## FOREIGN PATENT DOCUMENTS

0183444 6/1986 European Pat. Off. .

0183445 6/1986 European Pat. Off. .

60-220346 11/1985 Japan .

1247493 9/1971 United Kingdom .

1252418 11/1971 United Kingdom .

1398979 6/1975 United Kingdom .

## OTHER PUBLICATIONS

Research Disclosure No. 12443, *Research Disclosure*, vol. 124, 1974, Kenneth Mason Publications Ltd., Hampshire, England.

Research Disclosure No. 17643, *Research Disclosure*, vol. 176, 1978, Kenneth Mason Publications Ltd., Hampshire, England.

Primary Examiner—Paul R. Michl

Assistant Examiner—Mark R. Buscher

Attorney, Agent, or Firm—Richard E. Knapp

[57]

## ABSTRACT

Novel pyrazoloazole couplers comprise an aryl or heterocyclic group having, in at least one of the ortho positions to the carbon atom (A) that is bonded to the pyrazoloazole nucleus, a substituent (B) that enables the pyrazoloazole coupler to form a magenta dye that has increased stability and has absorption controllably shifted, that is shifted hypsochromically relative to a dye formed from a similar coupler lacking substituent (B). These couplers are useful in photographic silver halide materials and processes.

6 Claims, No Drawings

PHOTOGRAPHIC SILVER HALIDE MATERIALS  
AND PROCESS COMPRISING A  
PYRAZOLOAZOLE COUPLER

This application is a continuation-in-part of Ser. No. 171,061 filed Mar. 21, 1988, now abandoned, which is a division of Ser. No. 023,517 filed Mar. 9, 1987, now abandoned.

This invention relates to novel pyrazoloazole couplers and to photographic silver halide materials and processes using such couplers enabling formation of a magenta dye that has a desired shift in hue and increased stability.

Color images are customarily obtained by reaction between the oxidation product of a silver halide color developing agent and a dye forming coupler. Pyrazolone dye forming couplers are useful for forming magenta dye images; however, pyrazoloazole couplers represent another class of couplers that are useful for this purpose. Examples triazole couplers, such as 1H pyrazolo[3,2-c]-s-triazole couplers are described in, for example, U.S. Pat. Nos. 4,443,536; 4,540,654 and 4,777,121; and U.K. Patent Nos. 1,247,493; 1,252,418 and 1,398,979.

While such magenta dye forming couplers are useful in photographic silver halide materials and processes, many of such couplers provide dyes that do not have the desired properties. Pyrazolo azole couplers, particularly pyrazolotriazole couplers, often form magenta dyes that fall short of desired aims in hue and stability. For example, it has been found that pyrazolotriazole couplers typically form magenta dyes having hues that are shifted hypsochromically relative to the desired hues of dyes formed from pyrazolone couplers. It has also been found that aryl groups on the pyrazoloazole nucleus, for example, an unsubstituted phenyl group in the 3- or 6-position of a 1H-pyrazolo[3,2-c]-s-triazole, will enable formation of magenta dye having less than desired stability and a hue shifted bathochromically too far for most purposes for conventional photography.

It has also been desirable to provide a pyrazoloazole coupler that forms a magenta dye by reaction of the coupler with an oxidized silver halide color developing agent wherein the magenta dye has increased stability and the photographic sensitivity is not impaired. It has been desirable to provide such dyes that have with increased stability and a narrower absorption half band width (HBW) to improve hue purity and color saturation.

It has been found that a novel dye forming pyrazoloazole coupler enabling the described advantages has an aryl or heterocyclic group comprising a carbon atom (A) that is bonded to the pyrazoloazole nucleus, wherein the aryl or heterocyclic group comprises a substituent (B) in at least one position ortho to the carbon atom (A), and wherein the substituent (B) enables the dye formed upon reaction of the pyrazoloazole coupler with an oxidized silver halide color developing agent to have increased stability and controllably shifted absorption. The term controllably shifted absorption means that the dye formed from the pyrazoloazole coupler of the invention has an absorption shifted hypsochromically relative to a dye formed from a similar coupler lacking substituent (B).

Such dye forming couplers are particularly useful in photographic silver halide materials and processes. The substitution in the ortho position of the aryl or hetero-

cyclic group on the pyrazoloazole coupler causes the unexpected shifts in the hue of the dye formed from the pyrazoloazole coupler and enables formation of a dye having increased stability that is particularly useful in such materials and processes.

Pyrazolotriazoles are particularly useful pyrazoloazoles. Such pyrazolotriazoles include, for example, a 1H-pyrazolo[2,3-b]-1,2,4-triazole. A 1H-pyrazolo[2,3-b]-1,2,4-triazole can also be named as a 1H-pyrazolo[1,5-b]-1,2,4-triazole. The latter nomenclature has been used in the photographic art in, for example, U.S. Pat. No. 4,540,654. The ortho substituted moiety containing carbon atom (A), as described according to the invention, in the case of a pyrazolo[2,3-b]-1,2,4-triazole is in the 2- or 6-position and in the case of a pyrazolo[3,2-c]-s-triazole is in the 6- or 3-position.

It is believed that the steric constraints within the coupler molecule caused by the ortho substituent (B), at least in part, enables the described advantages. For example, it is believed that the 3- or 6-positions of a 1H-pyrazolo[3,2-c]-s-triazole coupler are most sensitive toward hue shifts of the dye formed by changes in substitution. Placement of an electron withdrawing group at the 6-position typically shifts the hue of the dye formed bathochromically. It was surprisingly found that the ortho substituent on the 6- or 3-position aryl or heterocyclic group caused the dye formed from the coupler to be shifted hypsochromically relative to the dye formed from the unsubstituted coupler by forcing the 6- or 3-substituent, particularly a 6-phenyl substituent, out of the plane of the pyrazolotriazole chromophore by steric constraints. Although the ortho group on the 6- or 3-substituent may in some cases reduce the oxidative coupling reactivity of the coupler, this reduced coupler activity can be increased by other means, such as by making the coupler more hydrophilic, for example by adding at least one water solubilizing group to the coupler. The shift of dye hue formed can be controlled by changing the groups on the 6- or 3-position substituents. The invention accordingly enables tailoring of the dye hue of a dye from a pyrazoloazole coupler to the desired wavelength.

Pyrazoloazole couplers according to the invention have an aryl or heterocyclic group represented by



wherein

$R_1$  is substituent (B), as described, preferably unsubstituted or substituted alkoxy, such as alkoxy containing 1 to 30 carbon atoms, for example, methoxy, ethoxy, propoxy, butoxy, decyloxy and eicosyloxy; halogen, such as chlorine, bromine and fluorine; or alkyl, such as unsubstituted or substituted alkyl containing 1 to 30 carbon atoms, for example, methyl, ethyl, propyl, butyl, pentyl, and eicosyl; and Q represents the atoms necessary to complete an unsubstituted or substituted aryl or heterocyclic group.

$R_1$  can be any substituent that enables the hue of the dye formed from the pyrazoloazole coupler to be controllably shifted, that is shifted hypsochromically to a desired degree relative to the dye formed from a pyrazoloazole containing no such substituent. For ex-

ample,  $R_1$  is preferably an unsubstituted or substituted alkoxy or alkyl group, or halogen. Unsubstituted or substituted alkoxy and alkyl groups as  $R_1$  enable formation of dyes that have unexpectedly improved light stability.

When the described aryl or heterocyclic groups contain two substituents (B) ortho to the carbon atom (A) the dye formed from the pyrazoloazole coupler has improved dye stability compared to a dye formed from a pyrazoloazole coupler containing only one substituent (B) ortho to the carbon atom (A).

The aryl or heterocyclic group completed by Q can be any such group which enables the desired coupling activity of the coupler as well as desired dye hue and stability of the dye formed. Typically useful aryl groups are phenyl or naphthyl groups. Typically useful hetero-

the desired properties of the coupler, for example alkoxy groups, such as alkoxy groups containing 1 to 30 carbon atoms, including methoxy, ethoxy, propoxy, butoxy and alkyleneoxy groups. Other illustrative optional groups on the aryl or heterocyclic group include ethyl, propyl, butyl and pentyl; and, groups known to be useful on photographic couplers, especially a ballast group. Alkyl in this group means alkyl containing 1 to 30 carbon atoms, such as methyl, ethyl, propyl, butyl, pentyl, octyl, decyl, and eicosyl.

A preferred coupler containing such a ballast group is a pyrazolo[3,2-c]-s-triazole coupler containing a 2,4,6-triarylphenyl group, preferably a 2,4,6-trimethylphenyl group, bonded directly to the 3-position of the coupler wherein the 2,4,6-triaryl phenyl group contains in the 3- or 5-position of the phenyl group a



cyclic groups contain 5 or 6 members in the ring and are, for example, pyridyl, furyl, and thienyl groups.

In addition to the substituent (B) as described, the aryl or heterocyclic group containing carbon atom (A) contains 1 to 4 other groups that do not adversely affect

25 The phenylene groups in such a ballast group can be unsubstituted or substituted with groups known in the photographic art.

Illustrative examples of aryl groups containing substituent (B) are as follows:



-continued



-continued



-continued



A preferred group is:



Illustrative examples of heterocyclic groups containing substituent (B) are as follows:



-continued



The pyrazoloazoles can comprise another ballast group in addition to the preferred ballast group as described. A ballast group as described is an organic radical of such size and configuration as to confer on the coupler molecule sufficient bulk to render the coupler substantially non diffusible from the layer in which it is coated in a photographic element. Couplers of the invention may be attached to ballast groups, or to polymeric chains through one or more of the groups on the pyrazoloazole nucleus. For example, one or more coupler moieties can be attached to the same ballast group. Representative ballast groups include substituted or unsubstituted alkyl or aryl groups containing 8 to 32

carbon atoms. Representative substituents include alkyl, aryl, alkoxy, aryloxy, alkylthio, arylthio, hydroxy, halogen, alkoxy carbonyl, aryloxy carbonyl, carboxy, acyl, acyloxy, carbonamido, carbamoyl, alkylsulfonyl, arylsulfonyl, sulfonamido, and sulfamoyl groups wherein the alkyl and aryl substituents and the alkyl and aryl portions of the alkoxy, aryloxy, alkylthio, arylthio, alkoxy carbonyl, aryloxy carbonyl, acyl, acyloxy, carbonamido, carbamoyl, alkylsulfonyl, arylsulfonyl, sulfonamido, and sulfamoyl substituents containing 1 to 30 carbon atoms and 6 to 30 carbon atoms, respectively, can be further substituted with such substituents.

Particularly useful pyrazoloazole couplers are those that comprise a water solubilizing group for some photographic materials that enables increased reactivity of the coupler. For example, a particularly useful coupler is a pyrazoloazole, as described, comprising a substituent, such as a ballast group, comprising at least one carboxy group.

Illustrative pyrazoloazole couplers are represented by the formula:



wherein Q and R<sub>1</sub> are as described; and, Coup is a pyrazoloazole coupler nucleus, such as a 1H-pyrazolo[3,2-c]-s-triazole or 1H-pyrazolo[2,3-b]-s-triazole nucleus, preferably those pyrazoloazole couplers that enable formation of magenta dyes which have not only a maximum absorption that is controllably shifted but also increased stability, and have on Q a preferred ballast group represented by BALL.

Preferred 1H-pyrazolo[3,2-c]-s-triazole couplers are represented by the formula:



wherein R<sub>2</sub> and R<sub>3</sub> are individually hydrogen or a substituent wherein at least one of R<sub>2</sub> and R<sub>3</sub> is



wherein Q represents the atoms necessary to complete an unsubstituted aryl group, such as aryl containing 6 to 30 carbon atoms, for example, phenyl and naphthyl, or heterocyclic group, such as a 5- or 6-member heterocyclic group, for example, pyridyl, furyl and thiienyl; Z is hydrogen or a coupling off group; R<sub>4</sub> is a substituent that enables the maximum absorption of the dye formed upon reaction of the 1H-pyrazolo[3,2-c]-s-triazole coupler with an oxidized silver halide color developing

agent to be controllably shifted and enables increased dye stability;

$R_5$  is a substituent group that does not adversely affect the coupler;

BALL is a preferred ballast group as described; and,  $p$  is 0 to 4.

Particularly preferred couplers are 1H-pyrazolo[3,2-c]-s-triazole couplers represented by the formulas:



wherein

$R_9$  and  $R_{14}$  are hydrogen or a substituent that does not adversely affect the coupler, particularly alkyl, such as alkyl containing 1 to 30 carbon atoms, or aryl, such as aryl containing 6 to carbon atoms, or heterocyclic, such as a 5 or 6 member heterocyclic group, for example, pyridyl, furyl and thieryl;

$R_{10}$  and  $R_{12}$  are the same as  $R_1$ , that is substituent (B), as described, preferably unsubstituted alkoxy, such as alkoxy containing 1 to 30 carbon atoms, for example, methoxy, ethoxy, propoxy, butoxy, decyloxy and eicosyloxy; halogen, such as chlorine, bromine and fluorine; or alkyl, such as unsubstituted alkyl containing 1 to 30 carbon atoms, for example, methyl, ethyl, propyl, n-butyl, t-butyl and eicosyl;

$R_{11}$  and  $R_{13}$  are the same as  $R_5$ , as described, that is a substituent that does not adversely affect the coupler;

$q$  is 0 to 4;

$Z_1$  and  $Z_2$  are hydrogen or a coupling off group, as described. Especially preferred couplers are those within the above formulas wherein  $R_{10}$ ,  $R_{11}$ ,  $R_{12}$  and  $R_{13}$  are groups, such as alkoxy groups, that enable the magenta dye formed from the coupler to have increased stability.

Pyrazoloazole couplers, preferably pyrazolotriazole couplers, according to the invention can be used in ways and for purposes that pyrazoloazole couplers have been used in the photographic art.

Pyrazoloazole couplers, particularly, pyrazolo-triazole couplers according to the invention are prepared by the general methods of synthesis described in the art, such as in *Research Disclosure*, August 1974, Item No. 12443 published by Kenneth Mason Publications, Ltd., The Old Harbourmaster's, 8 North Street, Emsworth, Hampshire PO10 7DD, England and U.S. Pat. No. 4,540,654. An illustrative synthesis scheme I is as follows:



10

15

20

25

30

40

45

55

60



( $Z_4$  is H (Compound E) or  $-SCOCH_3$  (compound E<sup>1</sup>))



wherein  $R_2$ ,  $R_3$ , and  $Z_4$  are as described.

In this illustrative synthesis scheme I a methanol or ethanol solution of a bromoketone (B) and a triazole (C) is refluxed 1 to 20 hours to produce triazolothiadiazine (D). The product is neutralized with sodium carbonate. A thermal extrusion of sulfur from the triazolothiadiazine with concurrent ring contraction is carried out by procedures described in *Research Disclosure*, August 1974, Item No. 12443. However, an improvement in the sulfur extrusion from triazolothiadiazine (D) is achieved by refluxing in acetic anhydride to produce compound (E<sup>1</sup>) wherein  $Z_4$  is  $SCOCH_3$  or by refluxing with triphenyl phosphine in acetic anhydride and toluene to produce compound (E) wherein  $Z_4$  is H accompanied by a small amount of compound (E<sup>1</sup>). Desired pyrazolotriazole (A) wherein Z is H is obtained by treating compound (E) with potassium hydroxide (KOH) or potassium carbonate (K<sub>2</sub>CO<sub>3</sub>) or by treating compound (E<sup>1</sup>) with concentrated hydrochloric acid/glacial acetic acid solution. The coupling off group, such as chlorine, can be added by procedures known in the organic synthesis art, such as described in, for example, U.K. patent specification No. 1,334,515. For example, chlorine can be added as the coupling off moiety by reaction of the pyrazolotriazole with N-chlorosuccinimide in dichloromethane. Particularly useful pyrazolotriazoles that can be prepared by this procedure are pyrazolotriazoles containing a t-butyl group in the 3-position and an aryl group, such as an ortho alkoxy or ortho alkyl substi-

tuted phenyl group, in the 6-position, with hydrogen or a coupling off group in the coupling position.

The intermediate triazole (C) is prepared by methods known in the organic synthesis art. For example, one process is illustrated by the following reactions:



Illustrative examples of synthesis of pyrazoloazole couplers, as described, are as follows: Synthesis Example A (Synthesis of Compound 6)

A solution of equimolar amounts of bromoketone (B, R<sub>3</sub> is 2-methyl-4- $\alpha$ -carbomethoxy undecyloxyphenyl) and triazole (C, R<sub>2</sub> is methyl) in methanol was heated to reflux until thin layer chromatography indicated starting materials were consumed. The mixture was concentrated in vacuo, then treated with 10% sodium carbonate solution and extracted with ethyl acetate. The separated organic layer was dried over magnesium sulfate and concentrated to give the desired product (D with R<sub>2</sub> and R<sub>3</sub> groups described above) as indicated by the following NMR spectrum:

NMR (CDCl<sub>3</sub>)  $\delta$ (ppm): 0.85 (m 3 H), 1.1–1.4 (broad s, 16 H), 1.9–2.1 (m, 2 H), 2.50 (s, 3 H), 2.55 (s, 3 H), 3.80 (s, 3 H), 3.85 (s, 2 H), 4.8 (t, 1 H), 6.8 (m, 2 H), 7.4 (d, 1 H).

To a solution of triazolothiadiazine (D) in toluene was added triphenylphosphine (4 molar equivalents), followed by acetic anhydride (2 molar equivalents). The resulting solution was heated to reflux for 2 hrs., cooled and concentrated in vacuo at about 50° C. The residue was immediately vacuum-chromatographed on silica gel G. Pure desulfurized product (E<sup>1</sup> with R<sub>2</sub> and R<sub>3</sub>

groups described above) was isolated in 65% yield and had the following NMR spectrum.

NMR (CDCl<sub>3</sub>)  $\delta$ (ppm): 0.85 (m 3 H), 1.1–1.4 (broad s, 16 H), 1.9–2.1 (m, 2 H), 2.45 (s, 3 H), 2.60 (s, 3 H), 2.65 (s, 3 H), 3.80 (s, 3 H), 4.8 (t, 1 H), 6.45 (s, 1 H), 6.45 (s, 1 H), 6.85 (m, 2 H), 7.5 (d, 1 H).

To a room temperature solution of pyrazolotriazole ester E<sup>1</sup> (4 mmol) in tetrahydrofuran (10 mL) was added 1.1 g (20mmol) potassium hydroxide in water (10 mL).

10 Sufficient methanol was added to keep the solution homogeneous. After stirring at room temperature for 2 hrs., the reaction mixture was cooled in an ice bath, neutralized with concentrated hydrochloric acid and extracted with methylene chloride. The organic layer

15 was filtered through anhydrous magnesium sulfate and concentrated in vacuo to give an off white solid. Pure product compound 6 (used in Example 6 of Table II) was obtained by trituration with hexane/diethyl ether, as evidenced by its melting point 154°–156° C., NMR, 20 and mass spectra;

NMR (CDCl<sub>3</sub>/DMSO-d<sub>6</sub>)  $\delta$ (ppm): 0.85 (m 3 H), 1.1–1.4 (broad s, 1 H), 1.9–2.1 (m, 2 H), 2.45 (s, 3 H), 2.55 (s, 3 H), 4.8 (t, 1 H), 5.8 (s, 1 H), 6.7–6.9 (m, 2 H), 7.5 (d, 1 H). M.S.: M<sup>+</sup> m/e 426.

25 Synthesis Example B—(Synthesis of compound 8)

To a solution of pyrazolotriazole compound 6 in methylene chloride (small amounts of CH<sub>3</sub>OH may be necessary to achieve complete solution) at room temperature was added 1 molar equivalent N-chlorosuccinimide in several portions. The reaction mixture was

30 then diluted with methylene chloride, washed with water and the organic layer filtered through anhydrous magnesium sulfate and concentrated in vacuo to give compound 8 as a solid product. Pure product having a melting point of 170–175° C. was obtained by trituration with hexane/diethyl ether and was verified by its NMR and mass spectra:

NMR (DMSO-d<sub>6</sub>/CDCl<sub>3</sub>)  $\delta$ ppm 0.85 (m, 3 H); 1.1–1.4 (broad s 16H); 1.9–2.1 (m, 2 H); 2.3 (s, 3 H); 2.55 (s, 3 H); 2.6 (s, 1 H); 4.65 (t, 1 H); 6.7–6.9 (m, 2 H); 7.35 (d, 1 H). FDMS: m/e 460.

35 Other 1H-pyrazolo[3,2-c]-s-triazole couplers can be prepared by procedures similar to those of synthesis Examples A and B.

40 Particularly useful illustrative couplers are pyrazolo[3,2-c]-s-triazoles as follows:



-continued



The photographic elements can be single color elements or multicolor elements. In a multicolor element, the dye forming coupler of this invention is typically associated with a green sensitized emulsion, although it could be associated with an unsensitized emulsion or an emulsion sensitized to a different region of the spectrum. Multicolor elements typically contain dye image forming units sensitive to each of the three primary regions of the spectrum. Each unit can be comprised of a single emulsion layer or of multiple emulsion layers sensitive to a given region of the spectrum. The layers of the element, including the layers of the image forming units, can be arranged in various orders as known in the art. In an alternative format, the emulsion sensitive to each of the three primary regions of the spectrum can be disposed as a single segmented layer.

A typical multicolor photographic element comprises a support bearing a cyan dye image forming unit comprised of at least one red sensitive silver halide emulsion layer having associated therewith at least one cyan dye forming coupler, a magenta dye image forming unit comprising at least one green sensitive silver halide emulsion layer having associated therewith at least one magenta dye-forming coupler of this invention and a yellow dye image-forming unit comprising at least one blue-sensitive silver halide emulsion layer having associated therewith at least one yellow dye-forming coupler. The element can contain additional layers, such as filter layers, interlayers, overcoat layers, subbing layers, and the like.

In the following discussion of examples of materials useful in the emulsions and elements of this invention, reference will be made to *Research Disclosure*, December 1978, Item No. 17643, the disclosures of which are incorporated herein by reference. This publication will be identified hereafter by the term "*Research Disclosure*".

The silver halide emulsions employed in the elements of this invention can be either negative working or

positive working. Examples of useful emulsions and their preparation are described in *Research Disclosure* Sections I and II and the publications cited therein. Examples of useful vehicles for the emulsion layers of elements of this invention are described in *Research Disclosure* Section IX and the publications cited therein

In addition to the couplers of this invention, the elements of the invention can include additional couplers, such as described in *Research Disclosure* Section VII, paragraphs D, E, F and G and the publications cited therein. These couplers can be incorporated in the elements and emulsion as described in *Research Disclosures* of Section VII, paragraph C and the publications cited therein.

The photographic elements of this invention or individual layers thereof, can contain brighteners (see *Research Disclosure* Section V), antifoggants and stabilizers (See *Research Disclosure* Section VI), antistain agents and image dye stabilizer (see *Research Disclosure* Section VII, paragraphs I and J), light absorbing and scattering materials) see *Research Disclosure* Section VIII), hardeners (see *Research Disclosure* Section XI), plasticizers and lubricants (see *Research Disclosure* Section XIII), matting agents (see *Research Disclosure* Section XVI) bleach accelerator and development modifiers (see *Research Disclosure* Section XXI) colored masking couplers, and competing couplers.

The photographic elements can be coated on a variety of supports as described in *Research Disclosure* Section XVII and the references described therein.

Photographic elements can be exposed to actinic radiation, typically in the visible region of the spectrum, to form a latent image as described in *Research Disclosure* Section XVIII and then processed to form a visible dye image as described in *Research Disclosure* Section XIX. Processing to form a visible dye image includes the step of contacting the element with a color developing agent to reduce developable silver halide and oxi-

dize the color developing agent. Oxidized color developing agent in turn reacts with the coupler to yield a dye.

Preferred color developing agents are p-phenylene diamines. Especially preferred are

4-amino-3-methyl-N,N-diethylaniline hydrochloride, 4-amino-3-methyl-N-ethyl-N- $\beta$ -(methanesulfonamido)ethylaniline sulfate hydrate,

4-amino-3-methyl-N-ethyl-N- $\beta$ -hydroxyethylaniline sulfate,

4-amino-3- $\beta$ -(methanesulfonamido)ethyl-N,N-diethylaniline hydrochloride and

4-amino-N-ethyl-N-(2-methoxyethyl)-m-toluidine di-p-toluenesulfonic acid.

With negative working silver halide this processing step leads to a negative image. To obtain a positive (or reversal) image, this step can be preceded by development with a non chromogenic developing agent to develop exposed silver halide, but not form dye, and then uniform fogging of the element to render unexposed silver halide developable. Alternatively, a direct positive emulsion can be employed to obtain a positive image.

Development is followed by the conventional steps of bleaching, fixing, or bleach fixing, to remove silver and silver halide, washing and drying.

The following examples further illustrate the invention.

#### EXAMPLES 1-15

Photographic elements were prepared by coating a cellulose acetate butyrate film support with a photosensitive layer containing a silver bromoiodide emulsion at 0.91 g Ag/m<sup>2</sup>, gelatin at 3.78 g/m<sup>2</sup>, and one of the couplers identified in Table I or Table II dispersed in one half its weight of tricresyl phosphate and coated at 1.62 mmoles/m<sup>2</sup>. The photosensitive layer was overcoated with a layer containing gelatin at 1.08 g/m<sup>2</sup> and bis vinyl sulfonylmethyl ether at 1.75 weight percent based on total gelatin.

Samples of each element were imagewise exposed

tions identified below then stopped, bleached, fixed and washed.

#### Developer Formulations:

|    |                                                                                        | D-1    | D-2    | D-3    |
|----|----------------------------------------------------------------------------------------|--------|--------|--------|
| 5  | 4-Amino-3-methyl-N,N-diethylaniline hydrochloride                                      | 2.45 g | —      | —      |
| 10 | 4-Amino-3-methyl-N-ethyl-N- $\beta$ -(methanesulfonamido)ethylaniline sulfate hydrate, | —      | 5.0 g  | —      |
| 15 | 4-amino-3-methyl-N-ethyl-N- $\beta$ -hydroxyethylaniline sulfate                       | —      | —      | 3.55 g |
| 20 | N- $\beta$ -hydroxyethyl aniline sulfate                                               | 2.0 g  | 2.0 g  | 2.0 g  |
| 25 | Potassium sulfite                                                                      | 30.0 g | 30.0 g | 30.0 g |
| 30 | Potassium carbonate (anhydrous)                                                        | 1.25 g | 1.25 g | 1.25 g |
| 35 | Potassium bromide                                                                      | 0.6 mg | 0.6 mg | 0.6 mg |
| 40 | 1% Solution in methanol of 5-nitro-1H-indazole                                         | 4.0 mL | —      | —      |
| 45 | Water to:                                                                              | 1.0 L  | 1.0 L  | 1.0 L  |
| 50 | pH adjusted to:                                                                        | 10.0   | 10.0   | 10.0   |

The well-defined magenta dye images produced in each element were evaluated by several tests and measurements. Dye hues were evaluated from spectrophotometric curves by measuring the maximum absorption peak (L<sub>max</sub>) normalized to a density of 1.0. The half-band width (HBW), an indication of hue purity, was measured as the width, in nanometers, of the spectrophotometric curve at one-half the difference between the maximum density and stain. Accelerated keeping tests on the dye image of initial density close to 1.0 gave the reported magenta density changes under the following conditions:

LF-3 - 3 week light fading under 5.4 Klux xenon simulated average north skylight.

WO-2 - 2 week "wet oven" dark keeping, 60° C./70% R.H.

DO-1 - 1 week "dry oven" dark keeping, 77° C./5% R.H. Comparison Coupler A:



through a graduated density test object and processed at 40° C. employing one of three color developing solu-

TABLE I

| Coupler  | X               | Y | LF-3 | WO-2 | DO-1 | L <sub>max</sub> | HBW |
|----------|-----------------|---|------|------|------|------------------|-----|
| Compr. A | (See structure) |   | -.56 | +.06 | n/a  | 556              | 82  |

TABLE I-continued



| Coupler  | X                                | Y                                | LF-3  | WO-2 | DO-1 | Lmax        | HBW |
|----------|----------------------------------|----------------------------------|-------|------|------|-------------|-----|
| Compr. B | H                                | H                                | -1.01 | +.07 | +.03 | 546 sh, 573 | 113 |
| Exmpl. 1 | Cl                               | H                                | -.62  | +.06 | +.01 | 569         | 92  |
| Exmpl. 2 | CH <sub>3</sub>                  | H                                | -.62  | +.05 | +.03 | 555         | 107 |
| Exmpl. 3 | CH <sub>3</sub>                  | CH <sub>3</sub>                  | -.30  | +.02 | +.01 | 557         | 81  |
| Exmpl. 4 | C <sub>2</sub> H <sub>5</sub>    | C <sub>2</sub> H <sub>5</sub>    | -.15  | +.05 | +.02 | 557         | 77  |
| Exmpl. 5 | C <sub>3</sub> H <sub>7</sub> -i | C <sub>3</sub> H <sub>7</sub> -i | *n/a  | *n/a | *n/a | 557         | 75  |

Developer D-1 was used to obtain Table I data. Absorption peak shoulder is indicated by "sh".

\*n/a means not available.

It can be seen from the data in Table I that an ortho substituent on an aryl ring attached to the 3-position of the pyrazoloazole coupler nucleus provides improved resistance to light fade and comparable or better resistance to fade under heat and humidity when compared to Comparison Coupler B which has no ortho substituent. In addition, a purer hue (narrower HBW) is also attained. Marked improvements in light fade and slightly more bathochromic and purer hues than provided by previously known Comparison Coupler A are achieved when two ortho substituents are present as in Examples 3-5.

Direct comparisons for a number of coupler structures bearing a 6-position aryl group are made in Table II between Comparison Couplers C, D, E, F, G, H

having no ortho substituent and inventive coupler Examples 6, 7, 8, 9, 10, 11, respectively, which have alkyl or alkoxy ortho substituents. It can be seen that in each case such ortho substitution results in improved resistance to light fade. Examples 13 and 15 show an even more remarkable improvement in light fade resistance when two alkoxy substituents are para to each other rather than meta to each other as in Examples 12 and 14, respectively. Dye hue improvements also generally result from ortho substitution according to the invention, allowing one to control the degree of bathochromic shift from the hue position of known Comparison Coupler A while maintaining a narrow half band width.

TABLE II



| Coupler   | Z <sub>5</sub> | R <sub>15</sub>                  | X                | (Y)n                                                 | LF-3 | Lmax        | HBW |
|-----------|----------------|----------------------------------|------------------|------------------------------------------------------|------|-------------|-----|
| Compr. A  |                |                                  |                  | (See structure)                                      | -67  | 554         | 88  |
| Compr. C  | H              | CH <sub>3</sub>                  | H                | 4'-Bal-la                                            | -83  | 535, 575 sh | 126 |
| Exmpl. 6  | H              | CH <sub>3</sub>                  | CH <sub>3</sub>  | 4'-Bal-la                                            | -36  | 563         | 102 |
| Compr. D  | Cl             | C <sub>4</sub> H <sub>9</sub> -t | H                | 4'-Bal-la                                            | -6   | 575         | 125 |
| Exmpl. 7  | Cl             | C <sub>4</sub> H <sub>9</sub> -t | CH <sub>3</sub>  | 4'-Bal-la                                            | -52  | 559         | 85  |
| Compr. E  | Cl             | CH <sub>3</sub>                  | H                | 4'-Bal-la                                            | -71* | 563         | 102 |
| Exmpl. 8  | Cl             | CH <sub>3</sub>                  | CH <sub>3</sub>  | 4'-Bal-la                                            | -43* | 559         | 93  |
| Compr. F  | Cl             | CH <sub>3</sub>                  | H                | 4'-Bal-lb                                            | -66  | 566         | 99  |
| Exmpl. 9  | Cl             | CH <sub>3</sub>                  | CH <sub>3</sub>  | 4'-Bal-1c                                            | -44  | 562         | 79  |
| Compr. G  | Cl             | Bal-2                            | H                | 4'-OCH <sub>2</sub> COOC <sub>2</sub> H <sub>5</sub> | -48  | 572         | 85  |
| Exmpl. 10 | Cl             | Bal-2                            | CH <sub>3</sub>  | 4'-OCH <sub>2</sub> COOC <sub>2</sub> H <sub>5</sub> | -45  | 569         | 74  |
| Compr. H  | Cl             | CH <sub>3</sub>                  | H                | 5'-Bal-3                                             | -82* | 577         | 89  |
| Exmpl. 11 | Cl             | CH <sub>3</sub>                  | OCH <sub>3</sub> | 4'-OCH <sub>3</sub> , 5'-Bal-3                       | -23* | 567         | 93  |
| Exmpl. 12 | H              | Bal-4                            | OCH <sub>3</sub> | 4'-OCH <sub>3</sub>                                  | -15  | 561         | 78  |
| Exmpl. 13 | H              | Bal-4                            | OCH <sub>3</sub> | 5'-OCH <sub>3</sub>                                  | -5   | 565         | 77  |
| Exmpl. 14 | Cl             | Bal-4                            | OCH <sub>3</sub> | 4'-OCH <sub>3</sub>                                  | -30  | 557         | 76  |

TABLE II-continued



| Coupler   | Z <sub>5</sub> | R <sub>15</sub> | X                | (Y)n                | LF-3 | Lmax | HBW |
|-----------|----------------|-----------------|------------------|---------------------|------|------|-----|
| Exmpl. 15 | Cl             | Bal-4           | OCH <sub>3</sub> | 5'-OCH <sub>3</sub> | -9   | 563  | 76  |

\*Data using developer D-2; all other data using developer D-3. (Absorption peak shoulder is indicated by "sh".)

Bal-1a is  $-\text{OCH}(\text{C}_{10}\text{H}_{21})\text{COOH}$

Bal-1b is  $-\text{OCH}(\text{C}_{10}\text{H}_{21})\text{COOC}_2\text{H}_5$

Bal-1c is  $-\text{OCH}(\text{C}_{10}\text{H}_{21})\text{COOCH}_3$

Bal-2 is  $-\text{CHO}$



### EXAMPLE 16

Photographic elements were prepared by coating a 35 cellulose triacetate film support with a photosensitive layer containing a silver bromoiodide emulsion at the 1x level equivalent to 0.882 g Ag/m<sup>2</sup>, gelatin at 3.71 g/m<sup>2</sup>, and one of the couplers in the table of results at the 1x level equivalent to 1.033 mmoles/m<sup>2</sup> dispersed in half its weight of tricresyl phosphate. The photosensitive layer was overcoated with a layer containing gelatin at 2.15 gm/m<sup>2</sup> and 1,1'-[methylenebis(sulfonyl)]bis-ethene (hardener) at 1.75 weight percent based upon total gelatin.

Samples of each element were imagewise exposed through a graduated density test object and processed using the commercial E-6 process and processing composition of Eastman Kodak Company, Rochester, N.Y. (with the exceptions that the first developer was shortened from 6 minutes to 4 minutes and the stabilizer bath step was omitted) at 37° C. using the following sequence to produce stepped magenta dye images:

|    |                     | Minutes |
|----|---------------------|---------|
|    | E-6 First Developer | 4.0     |
|    | Wash                | 2.0     |
|    | Reversal Bath       | 2.0     |
|    | Color Developer     | 6.0     |
|    | Conditioner         | 2.0     |
|    | Bleach              | 6.0     |
| 40 | Fix                 | 4.0     |
|    | Wash                | 4.0     |

The produced magenta dye images were evaluated by several tests and measurements. Densitometry of these images provided measures of maximum density (Dmax), shoulder speed (SPDS at a density of Dmax-0.3), and granularity (GRAN representing  $\sigma_D \times 1000$  at a density D=0.8). Spectrophotometry gave measures of the maximum wavelength of spectral absorption ( $\lambda_{max}$ ) and the width of spectral absorption at half peak height (HBW = half band width).

### Results

The results of the described tests are given in the 55 following table.

| Coupler | Coupler Laydown (moles) | Silver Laydown | Dmax | SPDS (Dmax-0.3) | GRAN D = 0.8 | $\lambda_{max}$ | HBW |
|---------|-------------------------|----------------|------|-----------------|--------------|-----------------|-----|
| C-16    | 1x                      | 1x             | 1.08 | 166             | 28.1         | 550             | 94  |
| A-16    | 1x                      | 1x             | 1.07 | 164             | 26.6         | 554             | 82  |
| B-16    | 1x                      | 1x             | 2.80 | 171             | 41.1         | 553             | 90  |
|         | 0.75x                   | 1x             | 2.28 | 165             | 34.6         | 552             | 89  |
|         | 0.5x                    | 1x             | 1.65 | 149             | 17.4         | 552             | 92  |
|         | 0.375x                  | 1x             | 1.24 | 132             | 18.2         | 551             | 96  |
|         | 0.25x                   | 1x             | 0.86 | 115             | 6.2          | 544             | 98  |
|         | 1x                      | 0.75x          | 2.47 | 171             | 40.7         | 554             | 92  |
|         | 1x                      | 0.5x           | 1.87 | 169             | 47.5         | 554             | 92  |
|         | 1x                      | 0.25x          | 0.90 | 149             | 56.8         | 555             | 96  |

-continued

| Coupler | Laydown | Silver  | SPDS | GRAN       |         |                 |     |
|---------|---------|---------|------|------------|---------|-----------------|-----|
| Coupler | (moles) | Laydown | Dmax | (Dmax-0.3) | D = 0.8 | $\lambda_{max}$ | HBW |
|         | 0.5x    | 0.75x   | 1.47 | 148        | 29.5    | 553             | 94  |
|         | 0.5x    | 0.5x    | 1.19 | 150        | 32.9    | 553             | 94  |

Compound A-16 (Invention)



Compound B-16 (Comparison)



Compound C-16 (Comparison)



These comparisons considered with data in the above identified application indicate that the color photographic element of the invention provides unexpectedly superior half band width with desired  $\lambda_{max}$  shift at matched sensitometry (Dmax) values without reduction of other desired results, particularly speed and granularity.

## EXAMPLE 17

Example 16 was repeated with the exception that the pyrazolo[3,2-c]-s-triazole coupler A-16 was replaced with a similar coupler except that the  $C_{10}H_{21}-n$  alkyl group of the coupler was replaced with methyl. The results provided a half-band width of 83 for this coupler.

55  
60

Example 16 was repeated with the exception that the pyrazolo[3,2-c]-s-triazole coupler A-16 was replaced with a similar coupler except that the  $C_{10}H_{21}-n$  alkyl group of the coupler was replaced with n-butyl. The results provided a half-band width of 83 for this coupler.

## EXAMPLE 18

The invention has been described in detail with particular reference to preferred embodiments thereof, but it will be understood that variations and modifications can be effected within the spirit and scope of the invention.

What is claimed is:

1. A photographic element comprising a support bearing at least one photographic silver halide emulsion

layer and a pyrazolo[3,2-c]-s-triazole coupler having a 2,4,6-trimethylphenyl group directly bonded in the 3-position of the coupler and a ballast group in the 3- or 5-position of the phenyl group wherein the ballast group is represented by the formula:



2. A photographic element comprising a support bearing at least one photographic silver halide emulsion layer and a pyrazolo[3,2-c]-s-triazole coupler having a group, directly bonded in the 3-position of the coupler, represented by the formula:

20



3. A photographic element comprising a support bearing at least one photographic silver halide emulsion layer and a magenta dye forming coupler represented by the formula:

40



4. A photographic element as in claim 1 comprising a red sensitive silver halide emulsion unit having associated therewith a cyan dye image providing material, a green sensitive silver halide emulsion unit having associated therewith a magenta dye image providing material, and a blue sensitive silver halide emulsion unit having associated therewith a yellow dye image providing silver halide material wherein the pyrazoloazole coupler is in at least one of said units.

5. A process of forming a magenta dye image in an exposed photographic element as defined in claim 1, said process comprising developing the exposed photographic element with a silver halide color developing agent.

6. A process of forming a magenta dye image in an exposed photographic element as defined in claim 3, said process comprising developing the exposed photographic element with a silver halide color developing agent.

\* \* \* \* \*

45

50

55

60

65